

**1**

3,502,503

**DESCALING OF TITANIUM AND ALLOYS  
THEREOF**

Louis J. Bartlo, Youngstown, and Octavian Berteia and  
Layne F. Plock, Warren, Ohio, assignors to Reactive  
Metals, Inc., a corporation of Delaware  
No Drawing. Filed May 10, 1967, Ser. No. 637,339

Int. Cl. C23g 1/28

U.S. Cl. 134—2

6 Claims

**ABSTRACT OF THE DISCLOSURE**

Process of descaling articles of titanium or titanium alloys which involves contacting the articles to be descaled with a substantially non-aqueous mixture of 35 to 50% potassium nitrate and 50 to 65% potassium hydroxide at a temperature in the range of 450° to 1000° F. to remove undesirable scale from the surfaces, thereafter rinsing and pickling in acid for residue removal.

This invention relates to descaling titanium. More particularly, the invention concerns a novel method of descaling titanium.

Oxide coatings and scale form on titanium and titanium alloys when heated to elevated temperatures. Scales that form on titanium surfaces at temperatures up to 1000° F. are generally thin and can be removed by acid pickling. However, heating titanium or its alloys for long periods of time or to high temperatures results in a formation of thick, adherent oxide scales that cannot be removed simply by acid pickling. Such scales must either be removed by mechanical means or by a chemical treatment designed to loosen the scale in normal acid baths or both.

Several commercial descaling baths are presently available for removal of scale on titanium alloys. However, all of the present commercial processes have characteristics that limit their usefulness as descaling media for a wide range of titanium products.

The titanium industry produces numerous products in a variety of thermal conditions. Presently available descaling processes do not have sufficient versatility to handle all of these products. For example, a number of age hardenable alpha-beta alloys are being produced in the solution-treated condition. These alloys require scale removal at temperatures below 600° F. to avoid altering metallurgical structure or properties. On the other hand, certain alpha alloys are fabricated at extremely high temperatures and have scales that are generally difficult to remove. Such alloys require high descaling temperatures for efficient scale removal. There is, therefore, a great need for a descaling media that can be operated efficiently over a broad temperature range.

A number of present commercial descaling baths are limited to operating temperatures above 800° F. because of their high melting points. One process referred to as the sodium hydride process has this disadvantage since it too is limited to fairly high operating temperatures, i.e. 650° to 750° F. An additional disadvantage of this bath is that it utilizes a reducing media and causes undesirable hydrogen contamination in most titanium alloys.

**2**

Low temperature aqueous descaling baths, such as disclosed in U.S. Patent No. 3,121,026, which require 10 to 20% water to maintain a liquidity, can be used for descaling. However, such baths have been found to be inefficient since they require excessive descaling time and repeated acid pickling to accomplish satisfactory scale removal. Moreover, these baths typically have relatively low maximum operating temperatures rendering them unsuitable for broad spectrum applications. The operating temperature limit of aqueous baths is usually about 475° to 500° F. which is too low for descaling many titanium materials.

The present invention provides a method of descaling titanium and titanium alloys which is operable over a wide temperature range, i.e. 450° to 1000° F., and which can therefore accommodate a wide variety of titanium products and which avoids the problem of hydrogen contamination as well. The invention involves an improvement in the process for treating titanium or titanium alloy articles having undesirable scale on the surface thereof for the purpose of removing same which comprises contacting said article with a substantially non-aqueous liquid bath consisting essentially of a mixture of 35 to 50% by weight potassium nitrate and 50 to 65% by weight potassium hydroxide at a temperature in the range of 450° to 1000° F., rinsing to remove the mixture and then treating with acid. The final acid treatment removes the last vestiges of scale and residue but the KOH—KNO<sub>3</sub> accomplishes primary scale removal. Several rinsing and acid pickling cycles may be performed if desired. In contrast to prior available descaling baths, the present invention provides a method of descaling various titanium products over a considerable temperature range and can, therefore, accommodate different products at different optimum conditions. Thus, for example, age-hardenable titanium alloys may be advantageously treated at temperatures between 500° and 600° F. and non-age-hardenable materials can be most effectively treated at temperatures of 750° to 800° F.

The following examples will illustrate the practice of the invention and its effectiveness under different conditions for treating a variety of titanium products. A series of samples were prepared in 1 by 2-foot panels of production material with typical mill scale. The scale producing conditions are described in Table I. The panel sections were treated in the preferred bath composition containing 55% KOH and 45% KNO<sub>3</sub> at various temperatures for varying times and the results are shown in Table II. The variety of materials treated successfully show the great versatility of the present invention. The production sheet materials were descaled in a 2 by 2 by 4-foot gas-operated steel tank which contained approximately 550 pounds of KOH and 450 pounds of KNO<sub>3</sub>. The descaling operation was carried out by immersing the sheets in the bath for the prescribed temperature and time. The sheets were then water rinsed and dipped in 10% H<sub>2</sub>SO<sub>4</sub> to insure removal of remaining residue and caustic. Following the sulfuric acid dip, the sheets were again water rinsed and immersed in 3 to 4% HF-25-30% HNO<sub>3</sub> acid bath for final cleanup.

TABLE I

|                      |        |                                                                                                    |
|----------------------|--------|----------------------------------------------------------------------------------------------------|
| Unalloyed Ti.....    | FHR    | Finish hot rolled.                                                                                 |
| Do.....              | FHR+EA | Finish hot rolled, electric furnace anneal: 1,350° F., 30 min., air cool.                          |
| Ti-4Al-3Mo-IV.....   | ST     | Solution treat: 1,625° F., 7 min., water quench.                                                   |
| Ti-5Al-2.5Sn.....    | FHR    | Finish hot rolled.                                                                                 |
| Ti-6Al-4V.....       | ST     | Solution treat: 1,650° F., 10 min., water quench.                                                  |
| Ti-6Al-4V.....       | CR+EA  | Cold rolled, electric furnace anneal: 1,475° F., 15 min., air cool.                                |
| Ti-6Al-4V.....       | FHR+EA | Finish hot rolled, electric furnace anneal: 1,475° F., 1 hr., furnace cool to 1,300° F., air cool. |
| Ti-8Al-1Mo-IV.....   | EA     | Electric furnace anneal: 1,450° F., 15 min., air cool.                                             |
| Ti-13V-11Cr-3Al..... | CR+EA  | Cold rolled, electric furnace anneal: 1,450° F., 15 min., air cool.                                |
| Ti-8Mn.....          | FHR+EA | Finish hot rolled, electric furnace anneal: 1,250° F., 1 hr., furnace cool to 900° F., air cool.   |

removed from each of the alloys. The optimum descaling conditions for various alloys are summarized in Table III.

TABLE III

| Alloy                | Condition <sup>1</sup> | Approximate Descaling Time in Minutes at— |         |         |
|----------------------|------------------------|-------------------------------------------|---------|---------|
|                      |                        | 550° F.                                   | 700° F. | 800° F. |
| Unalloyed Ti.....    | FHR                    | 5                                         | 5       | 5       |
| Do.....              | FHR+EA                 | 10-15                                     | 5-10    | 5-10    |
| Ti-4Al-3Mo-IV.....   | ST                     | 3-4 cycles <sup>2</sup>                   | —       | —       |
| Ti-5Al-2.5Sn.....    | FHR                    | 5                                         | 5       | 5       |
| Ti-6Al-4V.....       | ST                     | 2-3 cycles                                | —       | —       |
| Ti-6Al-4V.....       | CR+EA                  | 5-10                                      | 5       | 5       |
| Ti-6Al-4V.....       | FHR+EA                 | 10-15                                     | 5-10    | 5-10    |
| Ti-8Al-1Mo-IV.....   | EA                     | <5                                        | <5      | <5      |
| Ti-13V-11Cr-3Al..... | CR+EA                  | 2-3 cycles <sup>2</sup>                   | 10      | 5-10    |
| Ti-8Mn.....          | FHR+EA                 | 5                                         | 5       | 5       |

<sup>1</sup> See Table I for scaling conditions.

<sup>2</sup> A "cycle" consists of 10-min. descale, water quench, 5-min., 10% H<sub>2</sub>SO<sub>4</sub>, water rinse and dry. Last cycle is followed by 5-min. pickle in 3% HF-30% HNO<sub>3</sub>.

<sup>3</sup> Number of cycles is dependent on scale condition.

In addition to the excellent descaling characteristics of the bath, hydrogen pick up was found to be unusually low on all the titanium grades investigated. These results are illustrated in Table IV which reports the hydrogen data obtained prior to and following descaling.

TABLE IV

| Alloy                | Condition <sup>1</sup> | Hydrogen After Descaling and Pickling <sup>2</sup> |         |                                                    |                    |                    |                    |                   |
|----------------------|------------------------|----------------------------------------------------|---------|----------------------------------------------------|--------------------|--------------------|--------------------|-------------------|
|                      |                        | Base Hydrogen                                      |         | Hydrogen After Descaling and Pickling <sup>2</sup> |                    |                    |                    |                   |
|                      |                        | Avg.                                               | Range   | 500 F.,<br>40 min.                                 | 550 F.,<br>40 min. | 600 F.,<br>20 min. | 700 F.,<br>10 min. | 800 F.,<br>5 min. |
| Unalloyed Ti.....    | FHR                    | <sup>3</sup> 116                                   | 106-129 | 109                                                | 89                 | 106                | 123                | 114               |
| Do.....              | FHR+EA                 | <sup>4</sup> 66                                    | 50-79   | 55                                                 | 79                 | 80                 | 69                 | 65                |
| Ti-4Al-3Mo-IV.....   | ST                     | <sup>5</sup> 112                                   | 90-126  | 115                                                | 100                | 114                | —                  | —                 |
| Ti-5Al-2.5Sn.....    | FHR                    | <sup>6</sup> 71                                    | 59-92   | 65                                                 | 74                 | 63                 | 66                 | 73                |
| Ti-6Al-4V.....       | ST                     | <sup>6</sup> 92                                    | 54-124  | 94                                                 | 61                 | 95                 | —                  | —                 |
| Ti-6Al-4V.....       | CR+EA                  | <sup>6</sup> 44                                    | 40-50   | 40                                                 | 47                 | 44                 | 50                 | 44                |
| Ti-6Al-4V.....       | FHR+EA                 | <sup>8</sup> 63                                    | 37-102  | 57                                                 | 63                 | 47                 | 74                 | 57                |
| Ti-8Al-1Mo-IV.....   | EA                     | <sup>6</sup> 76                                    | 52-115  | 69                                                 | 79                 | 72                 | 70                 | 72                |
| Ti-13V-11Cr-3Al..... | CR+EA                  | <sup>6</sup> 116                                   | 114-123 | 118                                                | 116                | 105                | —                  | 117               |
| Ti-8Mn.....          | FHR+EA                 | <sup>4</sup> 103                                   | 84-124  | 92                                                 | 110/106            | 105                | 110                | 117               |

<sup>1</sup> See Table I for scaling conditions.

<sup>2</sup> Single analysis unless otherwise noted.

<sup>3</sup> Average of 11 analyses.

<sup>4</sup> Average of 12 analyses.

<sup>5</sup> Average of 10 analyses.

<sup>6</sup> Average of 9 analyses.

TABLE II

| Alloy                | Condition | Immersion Time, min. |     |     | Bath Temp., °F. | Percent Scale Removal |
|----------------------|-----------|----------------------|-----|-----|-----------------|-----------------------|
|                      |           |                      |     |     |                 |                       |
| Ti-6Al-4V.....       | CR+EA     | 20                   | 550 | 100 |                 |                       |
| Ti-6Al-4V.....       | ST        | 20                   | 550 | 100 |                 |                       |
| Ti-6Al-4V.....       | HR+EA     | 20                   | 550 | 100 |                 |                       |
| Ti-6Al-4V.....       | HR+EA     | 10                   | 700 | 100 |                 |                       |
| Ti-6Al-4V.....       | ST        | 10                   | 700 | 100 |                 |                       |
| Ti-6Al-4V.....       | HR+EA     | 5                    | 700 | 99  |                 |                       |
| Ti-6Al-4V.....       | ST        | 5                    | 700 | 100 |                 |                       |
| Ti-5Al-2.5Sn.....    | EA        | 20                   | 550 | 100 |                 |                       |
| Ti-5Al-2.5Sn.....    | EA        | 10                   | 700 | 100 |                 |                       |
| Ti-5Al-2.5Sn.....    | EA        | 5                    | 700 | 100 |                 |                       |
| Ti-8Al-1Mo-IV.....   | EA        | 20                   | 550 | 100 |                 |                       |
| Ti-8Al-1Mo-IV.....   | EA        | 10                   | 700 | 100 |                 |                       |
| Ti-8Al-1Mo-IV.....   | EA        | 5                    | 700 | 100 |                 |                       |
| Ti-8Mn.....          | EA        | 20                   | 550 | 100 |                 |                       |
| Ti-8Mn.....          | EA        | 10                   | 700 | 100 |                 |                       |
| Ti-8Mn.....          | EA        | 5                    | 700 | 100 |                 |                       |
| Ti-4Al-3Mo-IV.....   | ST        | 20                   | 550 | 75  |                 |                       |
| Ti-13V-11Cr-3Al..... | ST        | 20                   | 550 | 95  |                 |                       |
| Ti-13V-11Cr-3Al..... | ST        | 10                   | 700 | 100 |                 |                       |
| Ti-13V-11Cr-3Al..... | ST        | 5                    | 700 | 98  |                 |                       |
| Unalloyed.....       | EA        | { 10                 | 700 | 100 |                 |                       |
|                      |           | { 5                  | 700 | 100 |                 |                       |

Panels of Ti-6Al-4V, Ti-5Al-2.5Sn, Ti-8Al-1Mo-IV, Ti-8Mn, Ti-13V-11Cr-3Al and Ti-4Al-3Mo-IV were descaled at 550° F. for 20 minutes and rinse-pickled in 3-4% HF-25-30% HNO<sub>3</sub>. All materials descaled very well with the exception of the Ti-4Al-3Mo-IV and Ti-13V-11Cr-3Al which showed some scale remaining. Panels of unalloyed Ti, Ti-6Al-4V, Ti-5Al-2.5Sn, Ti-8Al-1 Mo-IV, Ti-8Mn and Ti-13V-11Cr-3Al were descaled at 700° F. for 5 and 10 minutes. The scale was completely

We have found that although the time articles are in the bath is not critical for achieving good quality surfaces, a preferred treating period of up to about 40 minutes is beneficial; however, the treating time is governed primarily by the tenacity of the scale being removed and the operating temperature of the bath. Low operating temperatures usually require the longest descaling time while treatment times of 3 to 5 minutes are common at operating temperatures of 700° to 850° F., where the nature of the titanium material permits the use of these temperatures.

An interesting observation in connection with the descaling of titanium alloys and products thereof is that the aqueous baths of the same materials, i.e. potassium hydroxide and potassium nitrate do not operate as effectively in descaling as the molten salt baths in accordance with the invention. Moreover, it has been further observed that the sodium hydroxide and sodium nitrate respectively are not effective substitutes for potassium hydroxide and potassium nitrate. This is demonstrated by the percent scale removal obtained in a series of tests on panels of different alloys treated in the descaling media at recommended temperatures. The results of these tests are described in Table V, which show that although certain alloys descale well in all baths, the descaling of some alloys was improved only when treated in accordance with the invention with a mixture of potassium nitrate and potassium hydroxide.

TABLE V

| Bath Composition, wt. percent | Temp., °F.                                   | Percent Descaled in 20 minutes |               |              |               |
|-------------------------------|----------------------------------------------|--------------------------------|---------------|--------------|---------------|
|                               |                                              | Ti-13V-11Cr-3Al                | Ti-4Al-3Mo-IV | Ti-6Al-4V    | Ti-16V-2.5Al  |
| 20 min.....                   | 75KOH-15KNO <sub>3</sub> -10H <sub>2</sub> O | 500 100%                       | 80%           | 100%         | 100%          |
| 20 min.....                   | 55KOH-35KNO <sub>3</sub> -10H <sub>2</sub> O | 500 100%                       | 50-85%        | 100%         | 100%          |
| 20 min.....                   | 55NaOH-45KNO <sub>3</sub>                    | 700 95%                        | 95%           | 100%         | 100%          |
| 20 min.....                   | 55KOH-45KNO <sub>3</sub>                     | 700 100%, 10 min.              | 100%, 20 min. | 100%, 1 min. | 100%, 20 min. |
| 20 min.....                   | 55NaOH-45NaNO                                | 700 70%                        | 90%           | 100%         | 100%          |

The unpredictability of the effectiveness of descaling media is illustrated in Table V above. However, in addition to the above, further evidence of the impossibility of satisfactorily predicting descaling effectiveness was obtained by tests conducted on a large number of experimental baths investigated in various combinations. Among the materials tested in descaling media for titanium and titanium alloys were the following:

|                                               |                                              |
|-----------------------------------------------|----------------------------------------------|
| NaCl                                          | K <sub>2</sub> S <sub>2</sub> O <sub>7</sub> |
| Na <sub>2</sub> CO <sub>3</sub>               | CuCl <sub>2</sub>                            |
| NaF                                           | SrCl <sub>2</sub>                            |
| Na <sub>2</sub> B <sub>4</sub> O <sub>7</sub> | Na <sub>2</sub> SO <sub>4</sub>              |
| KCl                                           | Cr <sub>2</sub> O <sub>3</sub>               |
| KBr                                           | CaCl <sub>2</sub>                            |
| KHSO <sub>4</sub>                             |                                              |

The baths containing the above materials in various combinations were screened in a similar manner to the tests described above but using smaller, i.e. 1-inch by 2-inch test coupons of several titanium sheet grades. The results indicated that potassium salts are superior to sodium salts but that only the mixtures of potassium hydroxide and potassium nitrate in the ranges specified, i.e. 50 to 65% KOH, 35 to 50% KNO<sub>3</sub>, were effective over the required temperature range for a sufficiently wide variety of titanium products.

We claim:

1. An improvement in a process of descaling articles of a metal from the group consisting of titanium and titanium alloys which avoids undesirable hydrogen contamination which comprises contacting said articles with a substantially non-aqueous mixture consisting of about 45% by weight potassium nitrate and about 55% by weight potassium hydroxide at a temperature in the range of 450° to 1000° F. to remove scale from the surfaces thereof, rinsing and pickling in acid for residue removal.

2. An improvement according to claim 1 comprising

treating articles of age-hardenable titanium alloy by contacting same with said mixture of potassium nitrate and potassium hydroxide at a temperature in the range of 500° to 600° F.

5 3. An improvement according to claim 1 comprising treating articles of non-age-hardenable titanium alloy by contacting same with said mixture of potassium nitrate and potassium hydroxide at a temperature in the range of 700° to 850° F.

10 4. An improvement according to claim 1 wherein said articles are in contact with said mixture of potassium nitrate and potassium hydroxide for up to about 40 minutes.

15 5. An improvement according to claim 1 wherein said titanium article is given more than one acid pickling treatment following contact with said potassium nitrate and potassium hydroxide mixture.

20 6. An improvement according to claim 5 wherein said titanium article is given a first acid pickling in dilute sulfuric acid, rinsed and then given a second acid pickling in a mixture of nitric and hydrofluoric acids.

#### References Cited

##### UNITED STATES PATENTS

|           |         |                |       |           |
|-----------|---------|----------------|-------|-----------|
| 2,458,660 | 1/1949  | Webster        | ----- | 134—3 XR  |
| 2,458,661 | 1/1949  | Webster et al. | ----- | 134—27 XR |
| 2,674,550 | 4/1954  | Dunlevy et al. | ----- | 134—3     |
| 2,826,539 | 3/1958  | Murtland       | ----- | 134—29 XR |
| 3,010,854 | 11/1961 | Satterfield    | ----- | 134—27    |
| 3,121,026 | 2/1964  | Beigay         | ----- | 134—2     |

MORRIS O. WOLK, Primary Examiner

J. T. ZATARGA, Assistant Examiner

35 U.S. Cl. X.R.

134—3, 27, 29; 252—156

UNITED STATES PATENT OFFICE  
CERTIFICATE OF CORRECTION

Patent No. 3,502,503

March 24, 1970

Louis J. Bartlo et al.

It is certified that error appears in the above identified patent and that said Letters Patent are hereby corrected as shown below:

Column 3, Table V, first column, line 4 thereof,  
"55NaOH-45NaNO" should read -- 55NaOH-45NaNO<sub>3</sub> --.

Signed and sealed this 29th day of December 1970.

(SEAL)

Attest:

Edward M. Fletcher, Jr.

Attesting Officer

WILLIAM E. SCHUYLER, JR.

Commissioner of Patents